

S. DAVIS.

PROCESS AND APPARATUS FOR THE MANUFACTURE AND HANDLING OF IMITATION METALLIC LEAF.  
APPLICATION FILED OCT. 26, 1921.

1,414,115.

Patented Apr. 25, 1922.

3 SHEETS—SHEET 1.



S. DAVIS.

PROCESS AND APPARATUS FOR THE MANUFACTURE AND HANDLING OF IMITATION METALLIC LEAF.  
APPLICATION FILED OCT. 26, 1921.

1,414,115.

Patented Apr. 25, 1922.

3 SHEETS—SHEET 2.



FIG. 2.



FIG. 4.



FIG. 3.

*Edward S. Davis* Inventor

S. DAVIS,

PROCESS AND APPARATUS FOR THE MANUFACTURE AND HANDLING OF IMITATION METALLIC LEAF.  
APPLICATION FILED OCT. 26, 1921.

1,414,115.

Patented Apr. 25, 1922.

3 SHEETS—SHEET 3.



# UNITED STATES PATENT OFFICE.

SEWARD DAVIS, OF MONTCLAIR, NEW JERSEY, ASSIGNOR TO CARL P. OLSON, OF IRVINGTON, NEW JERSEY.

## PROCESS AND APPARATUS FOR THE MANUFACTURE AND HANDLING OF IMITATION METALLIC LEAF.

1,414,115.

Specification of Letters Patent. Patented Apr. 25, 1922.

Application filed October 26, 1921. Serial No. 510,494.

To all whom it may concern:

Be it known that I, SEWARD DAVIS, a citizen of the United States, residing in the town of Montclair, county of Essex, and 5 State of New Jersey, have invented certain new and useful Improvements in Processes of and Apparatus for the Manufacture and Handling of Imitation Metallic Leaf, of which the following is a specification.

10 This invention relates generally to a process of manufacture of imitation gold leaf, silver leaf, or the like metallic leaf, and to apparatus for the practice of such process, and for handling the leaf as produced.

15 More particularly stated, it relates to the production of thin imitation metallic leaf of the kind usefully employed in the lettering and embellishing of book bindings by stamping or embossing same upon their cases 20 or covers. It has for its objects the production of such leaf as a continuous process at a comparatively rapid rate and with a minimum of manual labor and supervision; and more particularly, the production of a leaf 25 characterized by thinness, uniformity of texture, density and opacity. Further objects are: The automatic handling of the formed leaves and the interleaving thereof with a supporting tissue for packaging; and 30 finally, the recovery of the volatile solvent, such as amyacetate, customarily employed in making a solution of nitrocellulose, which, reconverted, becomes the binder of the fine metallic particles, termed generically bronze 35 powders, employed as the color component in such leaf manufacture.

My invention consists in certain novel steps in the above outlined processes and in certain novel means for practicing these 40 processes hereinafter more particularly set forth and described. These means comprise a leaf-forming apparatus adapted to supply a stream of leaf-forming mixture composed of nitrocellulose, dissolved in a volatile sol- 45 vent, and bronze powder suspended in said solution; of centrifugal feeding means adapted to concentrate the solids in said suspension along the line of delivery of the mixture to a continuously moving support 50 adapted to receive same as a coating; of pneumatic means adapted to thin said coating and to spread the same upon said support until the applied mixture is evenly distributed, and at the same time to increase

the rate of evaporation of the volatile sol- 55 vents by the application of the heated dry air supplied by said means under pressure; and of supplementing pneumatic means adapted to promote evaporation of the solvent and drying of the residue while serving 60 to compact the solids of the mixture in said coating while drying. My invention further consists in the provision of air-circulation means adapted to withdraw the drying medium supplied under pressure as continuous 65 currents of dry air to the coating as spread, and to pass same through a condenser whereby the volatile solvents employed are recovered. My invention finally 70 consists in handling means adapted automatically to wind the film as delivered from the support and to interleave it as wound, and in cutting means adapted to cut and stack the film ready for packaging in desired sizes. 75

My invention more particularly described, as to the method of film-formation, consists in the following steps: First, applying a leaf-forming solution of a binder, in which solution metallic particles in a fine state of subdivision are suspended, as a thin sheet delivered under centrifugal force to a revolving surface. To this end, the solution is revolved as a cylindrical column until the suspended particles respond to the force set 80 up by revolution and tend to become markedly less dispersed at the periphery of the column from which portion the delivery is effected. In this manner a maximum of 85 the metallic powders is applied to the leaf- 90 forming carrier and a leaf of high opacity and great covering capacity becomes attainable. Second, in applying a series of jets of air to the coating formed upon the continuously revolving carrier, the force and direction of the jets being so adjusted that the first acts substantially upon a plane tangential to the film and functions to spread the solution and drive off the volatile elements; the second acts substantially upon a chordal 95 plane of the revolving surface and tends to supplement the enforced evaporation while also tending to densify the residue and to compact the metallic particles therein by urging them into closer relation toward the 100 carrier; and the third acts substantially on a plane directed radially inward and tends to supplement the compacting action of its 105

predecessor, while also applying a drying temperature to the formed film.

In the drawings accompanying and forming a part of this specification, there is shown a preferred structural embodiment of means for attaining the objects sought. Like numerals of reference indicate like or corresponding parts throughout the several figures, in which Figure 1 shows in elevation, and principally in vertical section on the line I—I of Figure 2, a leaf-forming, winding and interleaving apparatus and condenser forming part thereof. Figure 2 is a plan view thereof. Figure 3 shows a horizontal section of the feed upon the line III—III of Figure 1. Figure 4 shows a horizontal section of the apparatus upon the line IV—IV of Figure 1. Figure 5 shows a vertical section on the line V—V of Figure 1. Figure 6 shows, in vertical section on the line VI—VI of Figure 1, the film winder and associated parts, including a clamp for the film on the winder positioned for removal of the filled winder. Figure 7 shows in elevation a winder adapted to produce a shorter leaf and the governor adjusting the interleaf supply roll thereto. Figure 8 corresponds to Figure 3, showing the adaptation of the feed means to the production of a narrower leaf. Figure 9 is a view in elevation of the loaded winder and illustrates the method of cutting the film, the cut film being shown in dotted lines as removed therefrom.

The like reference numerals indicate the like parts throughout the several figures, in which 1 is a motor, driving the gear 2 meshing with the gear 3, which drives a sprocket 4 and thereby the chain 5. This chain engages a wheel 6 whose shaft 7 is journaled in the bearings 8, 8, and has the hubs 9, 9, with spokes 10 supporting the drum 11 whose cylindrical surface constitutes the revoluble film-forming support. The motor, bearings, drum and their associated parts, as above described, are mounted upon a suitable frame-work 12, as shown. A portion of the drum and the film-forming means associated therewith, as hereinafter described, are enclosed in a suitable housing mounted upon said frame-work. The sprocket 4 is fixed to a main shaft 13 which extends to the opposite side of the frame, as shown in Figures 2 and 5, and carries a wheel 14, driving the belt 15 which drives the counter-shaft 16, belt 17, and stub-shaft 18 terminated by a crown-gear 19 meshing with a gear 20 upon the stirrer-rod 21 having the series of paddles 22 revolvably mounted within the mixer 23 containing the leaf-forming solution. This mixer has a delivery pipe 24 communicating with the horizontal pipe 25, shown in Figure 1, leading to the feeding-chamber 26, in which a stirrer 27 is rotated by the shaft 16 upon which it is mounted.

The feed-chamber 26 has an opening 27 adjacent the face of the film-forming drum whose vertical height is varied by the gate 28 slidably mounted between guides 29 and 30. The gate 28 is raised or lowered by the screw 31 having the adjusting nut 32. The opening 27 is adapted to be varied in width, as shown in Figures 3 and 7, by the gates 33, 34. On the shaft 7 is mounted a second sprocket 35 driving the chain 36 which meshes with a wheel 37 having the shaft 38 journaled at one end in an offset frame supporting the variable speed drive pulley system controlling the winding and interleaving apparatus, as shown in Figures 1 and 4 to 7. The shaft 38 carries a cylindrical pulley 39 driving the belt 40 which passes around the cone pulleys 41 and 42. A belt-shifter 43 is automatically controlled by the decreasing size of the paper feed roll 44 which is mounted upon the extension of the shaft carrying the cone pulley 42, in accordance with the increasing diameter of the interleaved film upon the winder 45 which is mounted upon an extension of the shaft carrying the cone pulley 41. This automatic control comprises a wheel 46 carried by an arm 47 fixed to a shaft 48 journaled in the standard 49. The shaft 48 is fixed to a sector 50 toothed to mesh with the teeth of a sector 51 fixed on the shaft 52 journaled in the standard 53. Fixed on the shaft 52 is the arm 54 terminated by the belt-engaging device 43 adapted automatically to move the belt 40 and to regulate the relative speeds of the roll 44 and winder 45. A shifter 55 for manually shifting the belt 40 is also provided. The spring 56 serves to hold the wheel 46 in pressing contact against the paper wound upon the roll 44. 57 is a fan driven from the pulley 58 and is adapted to draw air through the intake pipe 59 from the condenser 60, hereinafter to be described, and to deliver it by the pipe 61 through the heating chamber 62 containing the heating coils 63, around said coils and through pipe 64 to the slot-mouthed nozzles 65, 66 and 67 within the casing 68, at the surface of the drum 11 adjacent the film-receiving portion thereof. 69 are pipes extending on either side the drum and having their oppositely disposed openings 70 below the nozzles of the pipe 64 and within the casing 68, which casing forms a closure with that portion of the drum associated with the delivery of the film-forming solution. The pipe 69 leads the air saturated with the volatile constituents of such solution back to the condenser 60 and downward through the cooling chamber 70, containing water, to the series of communicating collecting chambers 71, 71, from which the condensed solvent may be drawn off by the cock 72. As will be apparent upon reference to Figures 1 and 4, the saturated air is caused to travel repeat-

edly through the cooling medium by a series of returning pipes in the chamber 70 opening into the communicating chambers 71, 71, circulation for the cooling medium being afforded by the pipes 73 and 74 opening into said chamber 70.

75 is a wetting roll mounted upon a pair of rolls 76 dipping into the wetting medium in the trough 77; the roll 75 is rotated by 10 its contact with the film-covered surface of the drum 11 and in turn rotates the dipping rolls 76; associated therewith is the delivery guide 78 which conducts the film 79 to the film winder 45. The spokes of this winder terminate outwardly in the hands 80, having the fingers 81, 81 and 82, 82. Between the fingers 81 and 82 are recesses adapted to receive the tool 83 having the parallel arms 84 adapted to grasp the interleaved film upon the 20 winder, a pair of tools being used, as shown in Figure 9, to hold the film while a cutting tool 85 is employed to sever the film between the fingers 82, 82, the groove therebetween permitting the tool 85 to seat therein. The clamping tool 83 is provided with pivoted handles adapted to be locked by the catch 86. Beneath the drum 11 is a brush 25 scraper 87 whose free ends 88 are in frictional engagement with the rotating surface 30 of the drum.

The operation of the apparatus is as follows:

The tank 23 is filled with a leaf-forming mixture. This mixture is preferably composed of soluble cotton dissolved in amylo-acetate, the amount of the solvent being in excess of that required to dissolve the nitro-cellulose, and bronze powder. The preferred proportions are, by weight, one ounce of 35 soluble cotton, dry, and eight ounces of bronze powder of the grade known as finest pale gold, or, substantially 10 per cent of cotton to 90 per cent of powder. This mixture is one that flows freely when the solvent of the cotton is in excess of the amount 40 needed to effect its solution. With this mixture, the speed of revolution of a drying drum five feet in diameter should be approximately five feet per minute, or  $\frac{1}{3}$  revolution per minute, with a drying temperature 45 between 150°-180° Fahr. The belt 5 having been adjusted to deliver the correct rate of drum-rotation, the feed gate 28 is adjusted by the screw 31 so that the opening 50 27 affords a minimum discharge to the drying drum 11. The film-forming periphery of this drum is preferably of hard, polished material. The temperature having been established by the coils 63 and 55 the suction fan 57 being in operation, the paper roll 44 is put in place and the governor 46 put in contact with its surface, the belt 40 being manually shifted till the 60 speed of the winder synchronizes with that of the drum in revolutions per minute.

The belt 40 is initially regulated by hand, so that, with a given solution the stirring and pumping may be more vigorous for a heavy solution, and the speed of the coating roll proportionally slower, the rates 70 adapted to produce the best results being better determined by the fluidity of the leaf-forming mixture. This mutual dependence is due to the discovery that a mixture high in bronze may be used to make 75 a denser leaf if the suspension of the bronze is maintained during the coating process. To this end, an active agitation of the mixture in the tank 23 is desirable. The mixture is caused to whirl as an entirety in 80 the feed chamber 26 until the metallic powders are thrown to the surface of the revolving column of solution before the gate 28 is lowered, thus a mixture high in bronze content is applied to the drying drum by 85 centrifugal force. This force is to be controlled so that its effect suffices to discharge the leaf-solution upon the drum in quantity sufficient to yield the minimum amount requisite to produce a continuous coating. 90

The deposited coating is first acted upon by an air current from the nozzle 67. The direction and pressure of the air discharged therefrom, due to the angle and width of the slot, acts primarily to spread the solution evenly over the drum's surface, thinning the coating and causing a homogenous covering. This covering then passes under the influence of the air-discharge from the nozzle 66, whose slot is narrower and directed at a more central inclination toward the drum. The effect of the air current is to supplement the action of the preceding current, and to cause a compacting of the metallic particles of the powder against the 100 drum's surface. The forming film next encounters the air-current discharged by the last nozzle whose slot is narrowest and directed radially inward against the drum. The effect of this current is to supplement the compacting action of the second current and to surface-harden the film. With the continued rotation of the drum, the film is carried to the wetting roll, the action of whose moisture causes the film to contract away from the drum. Thence it passes through the guide 78 to the winder 45 by which it is taken up together with the sheet of tissue from the paper roll and wound with the tissue interleaf as a continuous 110 length. The filled winder is removed when desired and replaced by an empty winder. The film and its interleaf are then cut, and lifted away from the winder by the gripping tools and the severed sheets laid back, 115 as shown in dotted outline in Figure 9. The tools are released and the film is ready for boxing in the form of a stack of metal leaves alternated with paper leaves, in the usual form in which such leaf is packaged 120 125 130

and marketed. Leaf of desired dimensions is producible, first, as to width, by the regulation of the slot of the feeding chamber by the gates 33 and 34, and second, as to length, by varying the diameter of the winder, interchangeable sizes of which may be provided, as illustrated in Figures 7 and 9, where winders of differing length of spokes are shown.

9 The reclamation of the volatile solvents employed is attained by the air circulation system illustrated. The fan supplies the heated air delivered within the casing 68 and withdraws it therefrom by the exhaust pipe 69 whose openings 70, 70 are within the enclosed casing 68. The withdrawn air is passed through the condenser and again circulated under the force of the fan, as described.

20 The economies attained by the automatic piling and interleaving of the film and by the recovery of the volatile solvents, together with the character and quality of the film produced and the speed of its production, realize the objects of my invention as hereinabove set forth, certain features of which I believe to be broadly new, as pointed out in the appended claims.

Having thus described my invention, I 30 claim:

1. The process of forming imitation metallic leaf as a continuous film, consisting in agitating a film-forming suspension of bronze powder, delivering same while undergoing agitation to a rotating distributor, delivering same therefrom by centrifugal force to a revolving surface, subjecting the coating so formed to a current of preheated air and removing the dried coating from said surface as a film of unlimited length.

2. The process of forming imitation gold leaf in unlimited lengths consisting in agitating a film-forming suspension of bronze powder, delivering same while undergoing agitation to a distributor, coating same upon a rotating surface, subjecting the coating so formed to a series of successive currents of preheated air, and removing the dried film from said surface as a continuous film.

3. In an apparatus for making imitation metallic leaf, the combination of a source of supply of a film-forming solution, means adapted to supply same continuously to the periphery of a revolving drum as a thin coating, said means comprising a feed-chamber having a slot parallel to the axis of the drum and adjacent the periphery thereof, means adapted to vary the width of said slot, and means adapted to cause the solution in said feed-chamber to rotate at a speed adequate to affect the metallic powders suspended in said solution centrifugally.

4. In apparatus adapted to form imitation metallic leaf as a continuous film, a source of film-forming solution containing a volatile solvent, means adapted to coat a predetermined width of the periphery of a revolving drum therewith, said means including a centrifugal feed delivery slot, said drum and means for driving same, a source of heated air, a plurality of slot-mouthed nozzles adjacent said drum, means adapted to cause the circulation of said air successively therethrough and through an enclosed channel leading from said heating source, over the periphery of said drum and through a condenser adapted to recover the volatile solvent.

5. In apparatus adapted to form imitation metallic leaf as a continuous process, a feed chamber and a horizontally revolving stirrer therein adapted to centrifugally feed a revolving drum surface adjacent thereto, means adapted to drive said stirrers and drum, means adapted to supply heated air under pressure to said revolving surface, the said means including a series of slotted vents extending across said drum surface, and said drum.

6. In apparatus adapted to form imitation metallic leaf as a continuous process, a gravity supply chamber and a vertically revolving stirrer therein, a feed chamber and a horizontally revolving stirrer therein adapted to centrifugally feed a revolving drum surface adjacent thereto, means adapted to drive said stirrers and drum, means adapted to supply heated air under pressure to said revolving surface, the said means including a series of slotted vents extending across said drum surface, and said drum.

7. In apparatus adapted to form imitation metallic leaf as a continuous process, a gravity supply chamber and a vertically revolving stirrer therein, a feed chamber and a horizontally revolving stirrer therein adapted to centrifugally feed a revolving drum surface adjacent thereto, means adapted to drive said stirrers and drum, means adapted to supply heated air under pressure to said revolving surface, the said means including a series of slotted vents extending across said drum surface, one of said slotted vents being adapted to direct a current of air at a tangent to said drum's surface, and said drum.

8. In apparatus adapted to form imitation metallic leaf as a continuous process, a gravity supply chamber and a vertically revolving stirrer therein, a feed chamber and a horizontally revolving stirrer therein adapted to centrifugally feed a revolving drum surface adjacent thereto, means adapted to drive said stirrers and drum, means adapted to supply heated air under pressure to said revolving surface, the said means including

- a series of slotted vents extending across said drum surface, one of said slotted vents being adapted to direct a current of air at a tangent to said drum's surface, another of said 5 slotted vents being adapted to direct a current of air perpendicularly to said drum's surface, and said drum.
9. In apparatus adapted to form imitation metallic leaf as a continuous process, a gravity supply chamber and a vertically revolving stirrer therein, a feed chamber and a horizontally revolving stirrer therein adapted to centrifugally feed a revolving drum surface adjacent thereto, means adapted to 10 drive said stirrers and drum, means adapted to supply heated air under pressure to said revolving surface, the said means including a series of slotted vents, one of said slotted vents being adapted to direct a current 15 of air at a tangent to said drum's surface, another of said slotted vents being adapted to direct a current of air perpendicularly to said drum's surface, and an intermediate slotted vent adapted to direct a current of 20
- air on a plane angularly disposed to the 25 planes of delivery of the other two slotted vents, and said drum.
10. In an apparatus adapted to form imitation metallic leaf from a liquid suspension of bronze powders, a revolving drum, a 30 centrifugal feed comprising a revolving stirrer in a chamber adjacent said drum, a horizontal slot in said chamber extending the width of said drum, means adapted to alter the width of said slot and means 35 adapted to vary the length of said slot.
11. In an apparatus adapted to form imitation metallic leaf from a liquid suspension of bronze powders, a revolving drum, a centrifugal feed comprising a chamber adjacent 40 said drum, a horizontal slot in said chamber extending the width of said drum, means adapted to alter the width of said slot and means adapted to vary the length of said slot, said centrifugal feed including a stirrer 45 adapted to cause the suspension in said chamber to revolve as a liquid column.

SEWARD DAVIS.